

Nov. 20, 1928.

1,692,521

H. E. STÜRCKE

MANUFACTURE OF CONTAINERS FOR COMPRESSED GASES

Filed May 8, 1924



Inventor

Herman E. Stürcke

By *Jack Richmond*

Attorney

## UNITED STATES PATENT OFFICE.

HERMAN E. STÜRCKE, OF PORT ORANGE, FLORIDA, ASSIGNOR TO WILLIAM WHARTON, JR. & COMPANY, INCORPORATED, OF EASTON, PENNSYLVANIA, A CORPORATION OF PENNSYLVANIA.

## MANUFACTURE OF CONTAINERS FOR COMPRESSED GASES.

Application filed May 8, 1924. Serial No. 711,877.

The manufacture of metal containers for compressed gases and the like, and particularly the testing of the containers, must conform to specifications and regulations of the 5 Interstate Commerce Commission. The test is a rigorous one and not only are there many wasters because of failure to meet the test requirements, but containers which fulfill such requirements may be so severely strained 10 thereby as to develop potential weaknesses which may manifest themselves disastrously at any time, thus making the containers unsafe in service.

With the view of correcting this evil, some 15 manufacturers, about ten or twelve years ago, instituted severe heat treatment of the steel as a preliminary step in the manufacture. The purpose of this was to produce steel of very high elastic limit and containers of comparatively thin walls and light weight. The 20 heat treatment consisted in heating the container to a temperature of about 1650 degrees F., then quenching for a few minutes in water heated to about 212 degrees F., or in a corresponding oil bath, followed by annealing at about 1200 degrees F. It has been demonstrated that some containers manufactured in this way are dangerously hard; that the steel lacks uniformity of quality even as to different sections of one container. Also, that 25 the annealing operation fails to sufficiently remove the heat stresses set up by the quenching. The stress strain diagram of this steel resembles that of cast steel. Many containers crack during or shortly after the quenching operation, the bottoms cracking off. There is no assurance that finished containers are 30 free from incipient cracks caused by quenching and not removed by annealing and not revealed by pressure test. In the average container for compressed gases the longitudinal stress is less than one-quarter of the circumferential stress. A container may therefore have 35 cracks running circumferentially through more than half the wall thickness without being materially affected by the pressure test. It is exceedingly difficult to control the heat treatment so that the containers will not turn out too hard. For instance, containers supposed to withstand a test pressure of 3300 40 pounds, and not much more, have been found to resist pressures of 4100 pounds, and more, without being stressed beyond the plastic point or the least stress intensity causing plas-

tic flow. Such containers obviously are too hard, toughness and ductility having been sacrificed for an unnecessarily high elastic limit.

Because of the defects, disadvantages, uncertainties and problems noted, there is a growing sentiment against heat treated containers, and personal observation, investigation and extended experimentation have convinced me that heat treatment is undesirable and unsuited for gas containers. 65

My invention, therefore, has for its principal objects, the production of containers for compressed gases unweakened by heat treatment; to provide a reliable and economical method of producing gas containers having desirable properties of strength and toughness, a sufficiently high elastic limit which, for the sake of accuracy, I prefer to call the plastic point and which shall be sufficiently ductile for specified test requirements; to provide a gas container whereof the qualities of strength and ductility are substantially balanced; and to provide for giving the container a cold pass without affecting more than the very top surface. Other objects and features of the invention will be discussed in the course of the detailed description and the invention will finally be defined in the claims hereto appended. 80

In the accompanying drawing, 85 Figure 1 is a chart or diagram of the steps employed in the practice of my invention, and

Figures 2, 3, 4 and 5 are graphic views of cylinders of the quenched type, showing average conditions of fracture under test or in service. 90

According to my invention, I start the manufacture of containers with a comparatively soft steel free of heat stresses and mechanical stresses. The containers may be formed in any usual manner, as by piercing or drawing or both. I then remove all incidental mechanical stresses by thorough annealing. The effect of this is to leave the steel 95 soft and ductile. Hence, there is no chance for lack of uniformity of quality, no chance for incipient cracks and no chance for excessive hardness. 100

The soft steel containers are subjected to predetermined interior pressure which stresses them beyond what I term the plastic point. Mechanical stresses are thereby set 105

up in the container walls, but not to an unnecessarily high degree. If the specified test pressure for a certain class of containers be, for example, 3,000 pounds, it is not necessary 5 or advisable to use a stretch pressure of more than 3,150 pounds or thereabout. I have shown in the Bulletin of the Compressed Gas Manufacturer's Association, Technical Series, that independent of the character of the 10 steel—as long as the modulus of elasticity does not vary materially from 30,000,000—there is a well defined relation between the volume of a container, its efficient (average) wall thickness, the internal pressure and volume 15 increase. I have likewise shown that if a test pressure is applied with reasonable speed to a container, and further pressure supply is cut off, the test pressure applied may remain constant, thereby proving that 20 the container has not been stressed beyond the plastic point. If, however, the applied test pressure recedes (not due to leaks or temperature changes) the extent of the recession gives a measure for the permanent non-elastic 25 condition of the container. If, therefore, the test pressure is applied with reasonable speed and further pressure supply cut off as soon as the maximum test pressure has been reached, the extent of the test pressure recession gives 30 a close indication whether or not the special container under test is in proper condition to be stretched by the predetermined stretch pressure. Excessive pressure recession indicates that the efficient wall thickness in general 35 is not as great as required or that the container has local defects, making it unfit for the stretch pressure intended. In this manner containers weak for any cause are eliminated previous to the completion of manufacture. 40 In other words, the preliminary pressure test decides what containers may be safely subjected to the predetermined stretch test without risking unduly hardening them. The preliminary test does not indicate that the container 45 could not be subjected to the stretch pressure and then finally stand the required test pressure, it is simply a check to sort out such containers which if subjected to the stretch pressure would turn out harder than 50 intended, less tough and less ductile. If the preliminary pressure test does not show excessive pressure recession, the full stretch pressure is turned on again and maintained for a brief period to stretch the container as 55 much as possible under the applied pressure.

Assuming that the containers have been stretched to the permissible predetermined limit, the next step is to remove the mechanical stresses or fatigues of the metal.

I have ascertained that this fatigue will disappear if the container is allowed to remain at rest for a time interval, depending upon the stress previously applied and the volume and form of the container, varying 60 from a few days to a few weeks. If it does

not interfere with the other operations it will therefore be sufficient to allow the container to remain at rest for the required period in order to remove the fatigue. If, after the rest period, the container is subjected to a test pressure of 3,000 pounds, it will be found to stand this test pressure without showing any or more than a negligible permanent expansion. The test pressure may be raised to 3,150 pounds, the previously applied stretch pressure, without showing more than a negligible permanent expansion. Furthermore, and this is very important, the total expansion of the container will now be proportionate to the pressure and entirely elastic; the pressure expansion diagram will be a straight line, proving absence of fatigue or mechanical stresses. The container has been strengthened to stand the required maximum test pressure with a minimum of loss in 70 toughness, ductility and shock resisting ability. 80

The rest period treatment may interfere with the other manufacturing operations or it may be desirable to put the containers through in a continuous manufacturing process. In this event the fatigue may be promptly removed by heating the container to a temperature which need not, but may exceed 212 degrees F. Any temperature between 212 degrees F. and ordinary annealing heat will remove the fatigue in a few minutes. (See J. Muir's Experiments, Encyclopedia Britannica, 11th edition, volume 25, page 90 1014.) Even at a temperature below 212 degrees F. the fatigue is removed in a short time. While, for my invention, it is not necessary to employ a temperature much above 212 degrees F., it is evident that the fatigue removal could be effected, say at 300 degrees F. with superheated steam. In short, while it is a merit of the invention that the fatigue removal can be accomplished at a temperature of substantially 212 degrees F., more or less, 95 I do not restrict myself to such, but may range between 212 degrees F. and 800 degrees F. 100

Containers produced by piercing or drawing ordinarily present a very rough surface 115 including longitudinal marks, ridges and depressions. Containers made according to my invention can be given a final "cold pass" by pressing them through an appropriate draw ring unheated or only slightly heated. This has the desired smoothing effect, but sets up mechanical stresses near the surface. These can be largely removed by an additional heating at a temperature not exceeding 800 degrees F. Nevertheless, the surface will remain slightly harder than the inner portions of the container walls, but the surface will be much less affected by corrosion and will ordinarily retain its smoothness 120 for many years. 130

Having described the nature and objects of the invention, I claim:

1. In the manufacture of containers for compressed gases, the method which consists in forming them from comparatively soft steel substantially devoid of heat and mechanical stresses, annealing them, subjecting the containers to internally applied pressure corresponding to the ultimate test pressure, and removing the mechanical stresses set up thereby.
2. In the manufacture of containers for compressed gases, the method which consists in forming them from comparatively soft steel substantially devoid of heat and mechanical stresses, annealing the containers, stretching them beyond the plastic point, and removing mechanical stresses or fatigue by heating the containers at a temperature below such as is calculated to produce any reduction of the elastic limit.
3. In the manufacture of containers for compressed gases, the method which consists in forming them from comparatively soft steel substantially devoid of heat and mechanical stresses, annealing them, applying a stretch pressure, and removing the fatigue induced thereby by heating the stretched containers to a temperature of 212 degrees F., more or less.
4. In the manufacture of containers for compressed gases, the method which consists in forming them from comparatively soft
5. In the manufacture of containers for compressed gases, annealing them, subjecting the annealed containers to predetermined stretch pressure, and removing mechanical stresses caused thereby by heating the stretched containers, for a short period, to a temperature ranging from substantially 212 degrees F. to 800 degrees F.
6. In the manufacture of containers for compressed gases, the method which consists in forming them from comparatively soft steel substantially devoid of heat and mechanical stresses, annealing them, subjecting the annealed containers to predetermined stretch pressure, removing the fatigue, and hardening the external skin of the containers.
7. In the manufacture of containers for compressed gases, that improvement which consists in stretching a container softer than required to stand the prescribed test pressure, and removing the fatigue by heating the stretched container to substantially 212 degrees F.

In testimony whereof I affix my signature.

HERMAN E. STÜRCKE